

[54] PROPELLANT COMPOSITION  
CONTAINING BERYLLIUM AND AN  
ENERGETIC DIFLUORAMINO  
CONTAINING BINDER

[75] Inventors: Kendall B. Randolph, Annapolis,  
Md.; Lewis B. Childs, Fairfax, Va.

[73] Assignee: The United States of America as  
represented by the Secretary of the  
Navy, Washington, D.C.

[22] Filed: Apr. 29, 1969

[21] Appl. No.: 823,241

[52] U.S. Cl..... 149/19.3, 149/19.4, 149/19.5,  
149/19.6, 149/19.91, 149/38, 149/42,  
149/43, 149/44, 149/61, 149/75, 149/76,  
149/85

[51] Int. Cl..... C06b 1/04

[58] Field of Search..... 149/109, 76, 45, 87, 42,  
149/46, 43, 92, 61, 19; 85, 20, 44, 38, 75

[56] References Cited

UNITED STATES PATENTS

3,332,811 7/1967 Guthrie et al..... 149/109

3,351,505 11/1967 Shapiro et al..... 149/44 X  
3,439,017 4/1969 Stevens ..... 149/44 X  
3,441,549 4/1969 Gardiner et al..... 149/44 X  
3,441,550 4/1969 Zimmerman..... 149/44 X  
3,447,323 6/1969 Allan ..... 149/36 X

Primary Examiner—Stephen J. Lechert, Jr.  
Attorney, Agent, or Firm—R. S. Sciascia; J. A. Cooke

[57]

ABSTRACT

A high energy composite propellant composition comprising a fuel component of beryllium, beryllium hydride and mixtures thereof in an energetic difluoramino containing binder material such as 2,3-bis(difluoramino)propyl acrylate (NFPA) addition polymerized with a vinyl monomer such as 2-hydroxyl propyl methacrylate and further plasticized with 1,2,3-tris[ $\alpha\beta$ -bis(difluoramino)ethoxy] propane (TVOPA), additional oxidizer such as ammonium perchlorate in amount sufficient to assure complete oxidation of the binder and fuel component and cured.

8 Claims, No Drawings

**PROPELLANT COMPOSITION CONTAINING  
BERYLLIUM AND AN ENERGETIC  
DIFLUORAMINO CONTAINING BINDER**

**BACKGROUND OF THE INVENTION**

This invention generally relates to novel propellant compositions and more particularly to an energetic composite propellant composition.

The development of high speeds and high thrusts is a major concern in the field of modern rocketry. In order to achieve these desired properties the use of high energy fuels is essential. Among such high energy fuels are included beryllium and beryllium hydride and mixtures thereof because these solid materials offer the ultimate in theoretical performance. Heretofore, however, the mainstream of propellant development to incorporate these high energy fuels has been in the area of the double-base formulations of nitrocellulose and nitroglycerin. Although, these formulations possessed certain advantages, combustion problems therein have resulted in significantly lower than theoretical performance efficiencies. These problems experienced by the prior art beryllium and beryllium hydride containing propellants are caused mainly by the formation of beryllium oxide (BeO) particles during the combustion process. For example, the BeO forms a coating about the desired beryllium particles and thereby inhibits the burning process since it is necessary to expend valuable heat energy in order to first melt the BeO layer before the burning of the desired beryllium fuel will begin. Furthermore, the presence of undue amounts of solid or liquid BeO particles in the propellant exhaust results in added reductions in the delivered specific impulse efficiencies of these prior art formulations due to the phenomena of lag-loss and two phase flow effects. The specific impulse efficiency of a propellant composition is the ratio of the actual specific impulse to the theoretical specific impulse.

Since beryllium and especially beryllium hydride are low density materials, the double-base propellants of the prior art incorporating these materials have also been of a low density. Low density propellant compositions are obviously disadvantages since they demand more operational space and thereby larger and heavier rocket motors in order to deliver an equivalent amount of energy as a higher density formulation. Moreover, because of this low density the density specific impulse values (which are a measure of the energy) of these prior art compositions are concomitantly lower than desired.

**SUMMARY OF THE INVENTION**

It is therefore an object of this invention to provide a new high energy composite propellant composition.

Another object of this invention is to provide a composite propellant composition which employs a beryllium containing fuel and which delivers a higher performance efficiency than those previously available.

Still another object of this invention is to provide a composite propellant composition which employs a beryllium containing fuel and possesses a higher specific impulse density than those previously available.

These and other objects are achieved herein by providing a composite solid propellant comprising an oxidizer, a beryllium, or beryllium hydride or mixtures

thereof fuel, in an energetic difluoramino polymeric binder matrix.

**DESCRIPTION OF THE PREFERRED  
EMBODIMENTS**

The composite solid propellants of this invention are prepared by the admixture of a fuel metal of either beryllium, beryllium hydride or mixtures thereof with an energetic difluoramino group containing polymeric binder matrix material and a solid oxidizing agent.

The beryllium, beryllium hydride and mixtures thereof fuel components of the present compositions are high energy materials. Generally, the quantity of fuel used in the compositions is dependent upon which of the fuel materials is employed. When free beryllium metal is utilized anywhere in the range of approximately 6 to 18 percent by weight of the total composition is found to be operable, however, for optimum results, it is advantageous to employ about 12 percent by weight of the total composition. In light of the very low density of beryllium hydride (BeH<sub>2</sub>), the amount which may be used in the composition is generally dependent upon the lowest overall density of the propellant composition which can be tolerated. For the purposes of this invention, it is desirable to employ BeH<sub>2</sub> from about 8 to about 25 percent by weight of the total composition, with optimum results being achieved at about a 15 percent by weight content. It is also desirable for the purposes of this invention to utilize mixtures of beryllium metal and beryllium hydride as the fuel component of the present compositions. When this is the case, approximately from about 7 to 17 percent by weight of this fuel mixture is used wherein the ratio of Be to BeH<sub>2</sub> may vary from 0 to 100 to 100 to 0 parts by weight, respectively.

The difluoramino group containing polymeric binders of the present invention are also high energy ingredients and yield a high theoretical performance. Besides improving the propellant density of the compositions, these energetic binders provide fluorine for the oxidation of the fuels to the corresponding gaseous fluorides. This formation of gaseous oxidation products, such as beryllium fluoride (BeF<sub>2</sub>), during the combustion process in place of some of the liquid and solid oxides, aids in the reduction of efficiency due to lag-losses and two phase-flow effects which are associated with the formation of solids and flow of condensed phases in the rocket or other propelled vehicle motor. In this respect, any energetic difluoramino group containing polymer material may be used as the binder material in the practice of this invention. These difluoramino binder materials are the addition polymerization products of an energetic difluoramino-vinyl containing monomer and another essentially non-energetic vinyl group containing monomer possessing hydroxy, carboxy, epoxide or anhydride functionality. An energetic difluoramino group containing plasticizer is further admixed with this addition polymerized product to complete the binder material. No further treatment of this binder is necessary prior to actual propellant mixing. Specifically, some of the energetic difluoramino containing monomers which are employed in the preparation of the addition polymerized product are 2,3-bis(difluoramino)propyl acrylate (NFPAA), poly[1,2-bis(difluoramino) 2,3-epoxy]propane (PBEP), 2,3-bis(difluoramino)propyl methacrylate (NFPMA)

and 1,2,4,5 tetrakis(difluoramino)amyl methacrylate (TAMA).

Some of the vinyl containing monomers possessing hydroxy, carboxy, epoxide or anhydride functionality which may be used for the purposes of this invention are, for example, 2-hydroxyl propyl methacrylate (HPMA), 2-hydroxyl propyl acrylate (HPA), acrylic acid (AA), methacrylic acid, glycidyl methacrylate, glycidyl acrylate, 2-hydroxyethyl acrylate, 2-hydroxyethyl methacrylate, maleic anhydride and the like. Among the energetic difluoramino containing plasticizers which are operable herein a 1,2,3-tris[ $\alpha$ ,  $\beta$ -bis(difluoramino)ethoxy] propane, hexakis(difluoramino) propylether (HPE), 1,2-di[2,2,3-tris(difluoramino)propoxy]-1,2-bis(difluoramino)ethane (OPE) and 1,2,4,5 tetrakis(difluoramino)amyl methacrylate and the like. The quantities of these hereinbefore identified monomers which are employed in the addition polymerization process are generally in the range of from about 80-97 percent by weight of the energetic difluoramino-vinyl monomer and from about 3 to about 20 percent by weight of the other vinyl monomer. Obviously the greatest amount of energetic monomer to the smallest amount of essentially non-energetic vinyl monomer is preferred in the addition polymerization process.

These addition polymerized products of the present invention have a number average molecular weight ( $\bar{M}_n$ ) percent from about 4,000 to about 28,000. Preferably the  $\bar{M}_n$  of the addition products are from about 6,000-7,000. The amount of energetic plasticizer which is admixed with the addition polymerization product to complete the binder material of the present invention may vary from about 50 to 80 percent by weight of the total binder material wherein optimum results are achieved in the vicinity of about 67 percent. The binder material comprises from about 35 to about 55 percent by weight of the total composition, preferably about 40 percent.

Subsequent to the admixture of the aforeidentified binder material with the remainder of the propellant ingredients, a cross-linking agent, in amounts of from about 0.5 to 5 percent by weight of the total propellant mixture is added and the mixture is cured. Among the cross-linking agents which are operable herein are any of the di- or trifunctional epoxides and isocyanates or any other materials which are conventionally employed as cross-linking agents for the curing of hydroxy, carboxy and anhydride functional polymers. More specifically, some of these are Unox 221, a difunctional cycloaliphatic epoxide product of the Union Carbide Corporation, (Formula I) Araldite 178 (Formula II) and 179 (Formula I) which are also difunctional cycloaliphatic epoxide products of the Ciba Corporation, any of the bisphenol A- epichlorohydrin epoxides, tolylene diisocyanate, hexamethylene diisocyanate and the like.



Formula I



Formula II

A solid organic or inorganic oxidizing agent which is compatible with the other ingredients of the propellant mixture and is capable of reacting with the matrix and fuel ingredients in combustion processes should be used for the purposes of this invention to supplement the energetic binder to assure complete propellant oxidation. Such suitable oxidizing agents include ammonium perchlorate, nitronium perchlorate, hydroxylammonium perchlorate and its derivatives, hydroxylammonium nitrate and its derivatives, potassium perchlorate, ammonium nitrate, and potassium nitrate. Also, suitable organic derivatives of nitrous acid, nitric acid, hydrogen peroxide, chromic acid, and perchloric acid can be employed as oxidizers, as well as RDX, HMX and nitramide. Also, when specific characteristics are required, two or more inorganic or organic oxidizing agents may be mixed together in the propellant composition.

Other additives normally incorporated into composite propellants may be added herein, such as curing catalysts, e.g., ferric acetylacetone, any of the various accelerators, burning rate catalysts, extenders, reinforcing agents, fillers and stabilizers, such as  $\text{Al}_2\text{O}_3$ .

The propellant compositions of this invention are also characterized by additional desirable properties not hereinbefore mentioned such as high burning rates, improved tensile properties, improved easy processing, thermal stability, long storage life. Moreover, the compositions of the present invention do not require stabilizing materials as 2-nitrophenyl amine and ethyl centralite as do prior compositions which deleteriously act to dilute the energetic materials of a propellant composition.

The general nature of this invention having been set forth, the following examples are presented as illustrations thereof. It will be understood that the invention is not limited to these examples but is susceptible to various modifications readily apparent to one of ordinary skill in the art.

#### Example 1

| Composition % weight |       |                                                                                                                                 |
|----------------------|-------|---------------------------------------------------------------------------------------------------------------------------------|
| 50                   | 9.66  | $\text{BeH}_2$                                                                                                                  |
|                      | 3.19  | Be                                                                                                                              |
|                      | 46.92 | ammonium perchlorate                                                                                                            |
|                      | 0.38  | hexamethylene diisocyanate                                                                                                      |
|                      | 39.85 | TVOPA/NFPA addition product (2/l)<br>(addition product is NFPA/HPMA,<br>90/10, intrinsic viscosity 0.28,<br>$\bar{M}_n$ 20,000) |

#### Example 2

| Composition % weight |       |                                                                                                                                 |
|----------------------|-------|---------------------------------------------------------------------------------------------------------------------------------|
| 60                   | 12.50 | Be                                                                                                                              |
|                      | 47.50 | ammonium perchlorate                                                                                                            |
|                      | 0.40  | hexamethylene diisocyanate                                                                                                      |
|                      | 39.60 | TVOPA/MFPA addition product (2/l)<br>(addition product is NFPA/HPMA,<br>90/10, intrinsic viscosity 0.28,<br>$\bar{M}_n$ 20,000) |

## Example 3

| Composition % weight |                                                                                                                           |
|----------------------|---------------------------------------------------------------------------------------------------------------------------|
| 15.27                | BeH <sub>2</sub>                                                                                                          |
| 44.73                | ammonium perchlorate                                                                                                      |
| 0.40                 | hexamethylene diisocyanate                                                                                                |
| 39.60                | TVOPA/NFPA addition product (2/l)<br>(addition product is NFPA/HPMA,<br>90/10, intrinsic viscosity 0.28,<br>$M_n$ 20,000) |

## Example 4

| Composition % weight |                                                                                                                  |
|----------------------|------------------------------------------------------------------------------------------------------------------|
| 12.86                | Be                                                                                                               |
| 47.04                | ammonium perchlorate                                                                                             |
| 0.10                 | Alon C (Al <sub>2</sub> O <sub>3</sub> )                                                                         |
| 1.44                 | Unox 221                                                                                                         |
| 38.56                | TVOPA/NFPA addition product (2/l)<br>(addition product is NFPA/AA, 96/4<br>intrinsic viscosity 0.34, $M_n$ 6600) |

at a temperature of about 50°-65°C for a complete day or more.

The preparation of the binder material follows the following general scheme, however, other procedures known to those skilled in the art may also be employed. The energetic monomer, such as NFPA, is added together with the other monomer, e.g., HPMA, and an initiator to the polymerization solvent. Polymerization occurs during a 24 hour reflux to produce the addition product. After polymerization the material is stripped of the solvent and the plasticizer is added thereto in solution. The solvent is then stripped by heat and vacuum and no further treatment is required until propellant mixing.

15 Table I below summarizes the densities, specific impulse and specific impulse efficiencies of some of the propellant compositions of the present invention.

Table I

| Composition | Isp (theoretical)<br>lbs/cu in. | Isp efficiency,<br>percent(measured)<br>Isp at 15° cone<br>angle |       |
|-------------|---------------------------------|------------------------------------------------------------------|-------|
|             |                                 | theoretical Isp<br>at 0° cone angle                              | angle |
| Example 1   | 0.0528                          | 299.1                                                            | 91.7  |
| Example 2   | 0.0628                          | 287.9                                                            | 94.0  |
| Example 3   | 0.0493                          | 304.8                                                            | 90.0  |
| Example 4   | 0.0639                          | 287.6                                                            | 95.3  |
| Example 5   | 0.0636                          | 287.4                                                            | 92.7  |

## Example 5

| Composition % weight |                                                                                                                  |
|----------------------|------------------------------------------------------------------------------------------------------------------|
| 12.86                | Be                                                                                                               |
| 47.14                | ammonium perchlorate                                                                                             |
| 1.44                 | Unox 221                                                                                                         |
| 38.56                | TVOPA/NFPA addition product (2/l)<br>(addition product is NFPA/AA, 96/4<br>intrinsic viscosity 0.34, $M_n$ 6600) |

Similarly, other compositions are prepared employing any of the other ingredients hereinbefore identified.

The compositions of Examples 1 to 5 and the other propellant compositions of this invention may be prepared by employing the following general scheme, however, other conventional methods may also be used. The binder material and the fuel metal component are premixed under vacuum conditions and at an elevated temperature of about 50°C. The oxidizing agent is added in increments with mixing under vacuum and elevated temperature conditions to this binder-fuel premix. After all of the oxidizing agent is added, the mixture is stirred further for about 2 hours longer. At this point, the cross-linking agent is added and the mixture is stirred for approximately 5 or 10 minutes under vacuum conditions. This total mixture is then cast and allowed to cure in an oven for about 24 hours or more

40 Many modifications of the present invention may be made without departing from the spirit or scope thereof.

What is claimed and desired to be secured by Letters Patent of the United States is:

## 1. A composite propellant composition comprising:

45 (1) a fuel component selected from the group consisting of beryllium, beryllium hydride, and mixtures thereof; (2) an energetic difluoramino group containing polymeric binder component which is comprised of the material resulting from the admixture of an energetic difluoramino group containing plasticizer and the addition polymerization product of an energetic vinyl difluoramino containing monomer with an essentially non-energetic vinyl monomer possessing hydroxy, or carboxy, or epoxide or anhydride functionality and a crosslinking agent, wherein the binder component is present in an amount of from about 35 to 55 weight percent of the total composition; and (3) a solid oxidizing agent component in amount sufficient to provide for complete oxidation of said binder and said fuel component.

55 2. The propellant composition of claim 1 wherein said solid oxidizing agent component is selected from the group consisting of ammonium perchlorate, nitronium perchlorate, hydroxylammonium perchlorate, hydroxylammonium nitrate, potassium perchlorate, am-

monium nitrate, potassium nitrate, cyclonite and homocyclonite.

3. The propellant composition of claim 1 wherein said fuel component is beryllium.

4. The propellant composition of claim 1 wherein said fuel component is beryllium hydride.

5. The propellant composition of claim 1 wherein said fuel component is a mixture of beryllium and beryllium hydride.

6. The propellant composition of claim 1 wherein said energetic plasticizer is selected from the group consisting of 1,2,3-tris[ $\alpha,\beta$ -bis(difluoramino)ethoxy] propane, hexakis (difluoramino) propyl ether, 1,2-di[2,2,3-tris (difluoramino) propoxy]-1,2-bis(difluoramino) ethane and 2,3-bis(difluoramino) propyl 2,2-dinitropropyl carbonate said energetic vinyl-difluoramino monomer is selected from the group consisting of 2,3-bis(difluoramino) propyl acrylate, poly[1,2-bis(difluoramino)2,3 epoxy] propane, 2,3-

10 bis(difluoramino propyl methacrylate and 1,2,4,5 tetrakis (difluoramino) amyl methacrylate and said essentially non-energetic vinyl monomer is selected from the group consisting of 2-hydroxypropyl methacrylate, 2-hydroxypropyl acrylate, acrylic acid, methacrylic acid, glycidyl methacrylate, glycidyl acrylate, 2-hydroxyethyl acrylate, 2-hydroxyethyl methacrylate and maleic anhydride and said cross-linking agent is selected from the group consisting of a difunctional cycloaliphatic diepoxide, and a diisocyanate.

15 7. The propellant composition of claim 1 wherein said addition polymerization product has a number average molecular weight of from about 4,000 to about 28,000.

15 8. The propellant composition of claim 7 wherein said number average molecular weight is from about 6,000 to about 7,000.

\* \* \* \* \*